

## UNITED STATES PATENT OFFICE

1,982,065

METHOD OF TREATING METAL DURING  
COLD ROLLINGGilbert H. Orozco, East Cleveland, Ohio, assignor  
to The Chandler Chemical Company, Cleve-  
land, Ohio, a corporation of OhioNo Drawing. Application December 30, 1933,  
Serial No. 704,795

10 Claims. (Cl. 153—10)

This invention relates to an improved method of treating the contact surfaces of metal stock to be formed and of the forming rolls during the cold rolling of metal shapes.

5 In the cold rolling of steel the metal to be formed is passed in cold condition through forming rolls and thereby bent to the desired shapes. In such operations, there is a surface slippage between the outer exposed faces of the metal and 10 the surfaces of the forming rolls and solutions must be provided for lubrication and to prevent overheating of the dies and consequent "sticking" of the material and dies. Again, it is necessary at the same time that the stock pass through the 15 rolls at substantially the rim speed of the rolls so that relative slippage between the stock and rolls in the direction of travel of the stock is eliminated. Due to such surface slippage, in cold rolling, the surfaces of the metal are often scarfed 20 or roughened, unless a suitable treatment is provided.

The customary practice has been to lubricate the rolls and the material with oils, greases, and different compounds containing the same, all of 25 which are generally known as "soluble oils", and comprise, in effect, aqueous emulsions of oils and greases. While such lubricants are fairly effective in preventing roughening of the materials being formed and also roughening of the rolls, 30 they are expensive and difficult to clean off of both the rolls and the material, and, in the case of the latter, require a two-stage cleaning process to prepare the work for commonly used rustproofing processes, such as by "Parkerizing" 35 or "Bonderizing". For example, it is necessary to clean the material with an alkali for removal of the oil and thereafter subject the same to a pickling bath. Even with these lubricants there 40 is a substantial loss in rejected material which has not reacted properly to the subsequent processes above mentioned or has become scarfed and roughened due to imperfect lubrication, imperfect cleaning, or both.

Again, with such lubricants, there is slippage 45 between the stock and rolls in the direction of travel of the stock so that additional scarfing and roughening results.

An object of the present invention is to effectively treat the surfaces of the metal stock and the rolls in connection with the cold rolling of steel or other metals so as to overcome these deleterious effects and disadvantages.

Another object is to effect these results in a 50 manner which renders subsequent cleaning of the

rolls and metal stock, other than by mere water rinsing, unnecessary.

Another object is to eliminate sticking of chips or flakes of steel or scale to the rolls or to the material with consequent roughening and scarfing of the surfaces thereof.

As exemplary of the process and the manner in which it is practised, and with no intent to limit the invention to the specific examples given, the invention will hereinafter be described in 65 connection with present manufacture of automobile tire rims of the demountable or drop center type, the application thereof to the cold rolling of other steel forms for fabrication being apparent therefrom.

In the manufacture of such rims, the common practice, after initially forming the same by cold rolling, is to complete the formation or fabrication by hand and also to rustproof or otherwise coat the same. One coating process generally 70 employed consists of polishing and cleaning the material and placing it in a solution of ferrous phosphate made from iron filings, about 1% of phosphoric acid, and water, the solution being boiled for approximately two hours and yielding 75 a light gray coating to the steel, which coating consists of iron phosphate, and is strongly adhesive. An oxidizing agent and catalyzing agent are added to the solution, usually manganese oxide, so that the coating is a basic ferric phosphate, 80 the ideal coating being one containing three of ferrous to one of ferric phosphate. This treatment is generally referred to as "Parkerizing".

When the materials are cold rolled, the surface is superficially hardened and is somewhat difficult 85 to attack by this process and consequently in order to shorten the time required and also to eliminate the sand or shot blasting steps of the "Parkerizing" process another patented process, commonly known as "Bonderizing", is employed, the 90 latter being more in the nature of chemically priming the material preparatory to enamelling.

If either of these processes are to follow the cold rolling process, it is apparent that great care 95 must be exercised to remove oils, chemicals and other foreign matter from the metal. If alkali cleaners having free caustic are used to remove the surface oils, they also must be removed before the "Parkerizing" or "Bonderizing" process is effective and consequently the material is usually 100 subjected to a water rinse.

Furthermore in the cold rolling of steel rims, for example, the stock is driven through the forming rolls by one of the rolls itself and if a grease lubricant is used, sufficient traction is not af- 110

forged between the driving roll and stock to pass the stock through the rolls without slippage.

All of these steps subsequent to the rolling are eliminated and better cooperation of the rolls and stock during rolling is afforded by the method with which the present invention is concerned. Experiments, followed by commercial success, have demonstrated that aqueous solutions of soluble alkalies, i. e. compounds, whose solution have a "pH" greater than 7, are very effective for providing efficient cooperation of the rolls and stock in the cold rolling process and may be readily removed by rinsing in water, and consequently their use eliminates the subsequent cleaning steps. Substantially any alkalies or alkali salts that are soluble in water may be used successfully though some have outstanding advantages over others. It should be borne in mind that as the "pH" increases upward from 7 the difficulty of removing the solution increases and it becomes increasingly dangerous to the workman because of its caustic properties. Furthermore, as the "pH" increases the necessity for pickling to remove the solution becomes more necessary. Solutions having a "pH" above but close to 7 are preferable, for example, a concentrated solution of borax would have a pH of 9.2 but a less concentrated solution having a pH of from slightly above 7 to about 8 is more desirable.

Solutions of sodium hydroxide, potassium hydroxide, sodium carbonate, sodium metasilicate and sodium tetraborate, the last of which is commonly known as "borax" and is defined chemically as  $\text{Na}_2\text{B}_4\text{O}_7 \cdot 10\text{H}_2\text{O}$ , are effective in concentrations between 1 ounce per gallon, which is approximately 1% concentration, as a lower limit, and saturation as an upper limit.

The mild alkalies having no free caustic, such for example, as sodium tetraborate are the most desirable and have many advantages particularly in that they are so easily removed from the metal and rolls by water rinse and will not deleteriously affect these or the hands of the workmen who subsequently handle the material before rinsing. Borax has an additional advantage in the fact that when forced or pinched into the pores of the metal, it will not deleteriously affect the "Parkerizing" or "Bonderizing" process, regardless of the concentration in which used. The solutions above are recited in the inverse order of desirability for treatment in general in cold rolling and may be used separately or mixed, and, if desired, with small additions of soap. For example, the borax may be used either plain or with small additions of about four parts of soap to ninety-six parts of borax, by weight, or four parts of tri-sodium phosphate and four parts of soap to ninety-two parts of borax.

The borax has, in addition to the advantages above enumerated, other advantages which make it most desirable. It can be quickly and easily removed from the work; its complete removal is not necessary as its presence does not interfere with the subsequent "Parkerizing" and "Bonderizing". Its use in commercial installations for a period of several months has given entire satisfaction both as to the actual results of rolling and convenience and safety in handling and the fact that it in no way deleteriously affects the forming rolls or the material or apparatus which is used in other operations on the material. Sodium hydroxide, on the other hand, requires an acid bath for removal by neutralization and cannot be rinsed out of the pores of the metal as readily by water.

As specific examples which have been found highly satisfactory in actual use but with no intent to limit the invention to the specific examples given, the following are cited:

1. An aqueous solution of  $\text{Na}_2\text{B}_4\text{O}_7 \cdot 10\text{H}_2\text{O}$  in concentrations of from about 1 to 20% by weight, the preferable concentration being about 6%, that is, 8 ounces per gallon of solution. 80
2. An aqueous solution of tri-sodium phosphate in concentrations of from about 1 to 20%, the preferred concentration being about 6%, that is, about 8 ounces per gallon of solution. 85
3. Aqueous solution of the following composition:

|                           | Concentration range | Preferred concentration | 90 |
|---------------------------|---------------------|-------------------------|----|
| Borax.....                | Percent<br>1 to 20  | Percent<br>6            | 95 |
| Tri-sodium phosphate..... | 0.2 to 5            | 0.5                     |    |
| Soap.....                 | 0.2 to 5            | 0.5                     |    |

It is most convenient to prepare the solution by thoroughly mixing the dry ingredients and dissolving portions of the mixture in water as required. For example, a dry mixture comprising borax 90%, tri-sodium phosphate 5% and tallow soap 5% may be thoroughly mixed dry and then dissolved in water in the proportions of about 8 ounces of the dry mixture to each gallon of solution thus making a solution containing approximately 6% of the mixture. This, however, is also effective between the limits of 1 to 20% concentration. These solutions can be used at any convenient temperature, depending upon the solubility of the salts used, as the temperature of the lubricants is of relatively small importance in the rolling process. It is obvious, however, that higher temperatures are required when the higher concentrations are used because of the limits of solubility of the constituents at lower temperatures, the solubility being greater at the higher temperatures. 100 105 110 115 120

It has been found that the effect of such treatment of the stock is sufficient to substantially eliminate scarfing and roughening of the material and yet the composition used in connection with the treatment is of such consistency that it will not act to hold foreign matter, such as scale and the like, on the surfaces of the forming rolls or on the material formed. 125

Further, the composition may be conveniently applied in the same manner as lubricants commonly used, and either on the rolls or the metal stock, or both, before or during the forming operation so that during the forming operation the surfaces are sufficiently coated. After forming, the metal is rinsed with water to remove the alkali composition. 130 135

Having thus described my invention, 135

I claim:

1. The method of treating the complementary contact surfaces of metal stock to be formed and forming rolls during the cold rolling of metal shapes comprising maintaining on said surfaces in liquid condition and during the forming operation an aqueous solution of mild alkali containing substantially no free caustic and the mild alkali being in excess of any other solid contained in the solution. 140 145

2. The method of treating the complementary contact surfaces of metal stock to be formed and forming rolls during the cold rolling of metal shapes comprising maintaining on said surfaces 150

- in liquid condition and during the forming operation an aqueous solution of mild alkali containing substantially no free caustic and substantially no organic matter.
5. 3. The method of treating the complementary contact surfaces of metal stock to be formed and forming rolls during the cold rolling of metal shapes comprising maintaining on said surfaces in liquid condition and during the forming operation an aqueous solution of mild alkali containing substantially no free caustic and free from soap in excess of 25% by weight of the alkali. 80
10. 4. The method of treating the complementary contact surfaces of metal stock to be formed and forming rolls during the cold rolling of metal shapes comprising maintaining on said surfaces in liquid condition and during the forming operation a non-saponaceous aqueous solution of mild alkali containing substantially no free caustic. 85
15. 5. The method of treating the complementary contact surfaces of metal stock to be formed and forming rolls during the cold rolling of metal shapes comprising maintaining on said surfaces in liquid condition and during the forming operation an aqueous solution of mild alkali containing a quantity of soap less than 20%, by weight, of the quantity of alkali. 90
20. 6. The method of treating the complementary contact surfaces of metal stock to be formed and forming rolls during the cold rolling of metal shapes comprising maintaining on said surfaces during the forming operation an aqueous solution of mild alkali containing substantially no 95
25. free caustic, and soap, said solution being of from 1 to 20% concentration and the soap content, by weight, being not in excess of 10% of the alkali content. 100
30. 7. The method of treating the complementary contact surfaces of metal stock to be formed and forming rolls during the cold rolling of metal shapes comprising maintaining on said surfaces during the forming operation an aqueous solution of mild alkali, comprising sodium tetraborate 1 to 20%, tri-sodium phosphate 0.2 to 5%, soap 0.2 to 5%. 105
35. 8. The method of treating the complementary contact surfaces of metal stock to be formed and forming rolls during the cold rolling of metal shapes comprising maintaining on said surfaces during the forming operation an aqueous solution of mild alkali, comprising borax 6%, tri-sodium phosphate 0.5%, and soap 0.5%. 110
40. 9. The method of treating the complementary contact surfaces of metal stock to be formed and forming rolls during the cold rolling of metal shapes comprising maintaining on said surfaces during the forming operation an aqueous solution containing sodium tetraborate as the principal solid ingredient contained in the solution. 115
45. 10. The method of treating the complementary contact surfaces of metal stock to be formed and forming rolls during the cold rolling of metal shapes comprising maintaining on said surfaces during the forming operation an aqueous solution containing tri-sodium phosphate as the principal solid ingredient contained in the solution. 120
50. 51. GILBERT H. OROZCO. 125
55. 60. 130
60. 65. 135
65. 70. 140
70. 75. 145
75. 80. 150